

Oct. 20, 1925.

1,558,005

D. FINLEY

CONSTRUCTION MATERIAL

Filed Aug. 18, 1921



FIG. 1

FIG. 2



FIG. 3



FIG. 5



FIG. 4

WITNESS

*A. E. Allay.*

INVENTOR

*DOZIER FINLEY*

BY

*White, Prost & Evans*  
his ATTORNEYS

Patented Oct. 20, 1925.

1,558,005

# UNITED STATES PATENT OFFICE.

DOZIER FINLEY, OF OAKLAND, CALIFORNIA, ASSIGNOR TO THE PARAFFINE COMPANIES, INC., OF SAN FRANCISCO, CALIFORNIA, A CORPORATION OF DELAWARE.

## CONSTRUCTION MATERIAL.

Application filed August 18, 1921. Serial No. 493,344.

To all whom it may concern:

Be it known that I, DOZIER FINLEY, a citizen of the United States of America, and a resident of Oakland, county of Alameda, and State of California, have invented a new and useful Construction Material, of which the following is a specification.

My invention relates to a covering unit such as a shingle or shake which has an 10 armoring plate of protective material applied to it.

The broad object of the invention is to provide an armored shingle characterized by the qualities of increased durability and 15 resistance to fire. Another object of the invention is the provision of a shingle so armored as to give the qualities desired but which is not thereby rendered difficult to apply nor unduly increased in weight, nor 20 otherwise altered so as to require materially different methods in packing or handling. Another object of the invention is to provide a shingle of the character described at slightly increased cost over that of the untreated 25 shingle and in which classes of timber not usually considered to be adapted for shingle making may be used with success. Another object is the provision of an armored shingle 30 which possesses all of the adaptability for artistic treatment found in the ordinary shingle.

My invention has many other objects and features of advantage, some of which the foregoing, will be set forth in the following 35 description of my invention. It is to be understood that I do not limit myself to the showing made by the said description, as I may adopt variant forms of my invention within the scope of the claim.

Referring to the drawings, Fig. 1 is a perspective view of a shingle made in accordance with my invention, a portion thereof being shown in section. Fig. 2 is an elevation of a fragment of a shingle drawn on an 40 enlarged scale and showing my method of interlocking the armoring plate with the wooden base. Figs. 3, 4 and 5 are views similar to Fig. 1, but illustrate modified 45 forms of my invention. In the drawings, portions are shown somewhat out of the proportion in order to more clearly indicate the 50 nature of my invention.

The characteristics and advantages of wooden shingles, which have given them 55 such a wide use, are well known, but the

wooden shingle has one serious shortcoming,—its high fire hazard. Primarily my invention is directed to curing this defect without materially altering the other qualities of the wooden shingle which have caused 60 its extensive use. I accomplish this purpose by applying to the exposed portion of the shingle a protective mat or shield or plate of durable and fire-resistant material having a suitable surface finish which lends 65 itself to artistic treatment. In the following description I shall use the term shingle to mean the ordinary shingle of commerce, the shake or any allied covering unit of 70 wood.

The first step in producing my armored shingle is to dip or brush it with a bituminous compound 2 of low melting point. The excess compound clinging to the shingle 75 3 is then drained away or scraped off, and the shingle passed thru a heated zone for a short period so as to drive in the compound. This priming coat of low melting point bituminous compound impregnates the wood to a small degree and also fluxes 80 with the much higher melting material of the protective plate 4 which is applied over it. Thus being partly sunk into the wood and partly fluxed with the super-added material it locks the latter to the former acting 85 as a root for the protective or armoring plate. In the drawings I have illustrated this penetration by extending the section lines of the priming coat a short distance 90 into the body of the shingle.

The bituminous compound forming the priming or root coat may consist of any of a wide range of materials used singly or mixed together. It may be asphaltum, 95 heavy crude petroleum, refined coal tar, candle tar, pine tar, or other substances of a generally similar nature. While I have mentioned the priming coat as a bituminous compound, other compounds not usually classed as bituminous may be used, as for instance, a mixture of resin and resin oil. Oils such as linseed oil may be mixed with the compound employed. Antiseptic materials such as creosote may also be mixed 100 with the compound with the object of preserving the wood from decay. Bituminous paint such as asphaltum dissolved in benzine 105 may be used. I prefer however to use a liquid asphaltum because of its relative cheapness and good working qualities. The 110

grade known as "L oil" or "L asphaltum" produced from California crude petroleum gives good results.

In order to attach additionally, the armor-  
5 ing plate to the wood, I prefer to raise upon the surface to be coated, barbs 6 of the base fiber as shown in Fig. 2. Preferably this is done after the priming coat has been applied. These projections or barbs are conveniently  
10 formed by a suitable sharp tool driven into the surface of the wood, and about thirty-six per square foot has been found sufficient. Of course the barbs should be raised in such a direction that they tend to prevent the  
15 coating from sliding toward the butt or exposed end of the shingle.

The armoring plate 4 of protective material is next added, and preferably consists of an asphaltum produced from the refining of crude petroleum and having a penetration of 18 according to the method of the American Society for Testing Materials, using the standard needle with 100 grams weight for five seconds at 77° Fahrenheit, 20 and having a melting point of 200° Fahrenheit by the ball and ring method. 100 pounds of such asphaltum is heated in a container to a temperature of about 400° Fahrenheit and maintained at that temperature while 80 pounds of crushed limestone, 25 of a fineness to pass thru an 80-mesh screen, and 15 pounds of asbestos fiber, of the grade suitable for making asbestos paper, is thoroughly mixed in. The mixture thus prepared and at the temperature of approximately 400° Fahrenheit is applied by any suitable means over the predetermined area of the shingle so that a plate of the protective material preferably about 1/16 of an inch in thickness is formed. It will be seen from an inspection of Fig. 2, that the material flows about the barbs 6 and into the recesses formed by the raising of the barbs 30 so that the armoring plate is literally interlocked with the wooden base. Preferably the armoring plate of material is extended over the butt of the shingle as shown in Fig. 1, and under the end of the butt.  
35 While the coating is still plastic and adhesive, owing to the elevated temperature, granular mineral matter is sprinkled on the surface and embedded therein by pressure rollers. This mineral matter may be crushed slate, flint, limestone, silica, jasper, serpentine, asbestos or any other material of desirable color and hardness. Such mineral matter if of actual granular form may be conveniently of such size that it will entirely pass thru a 12-mesh screen and be retained on a 24-mesh screen. If of fibrous nature the mineral matter should all pass thru a 4-mesh screen and be retained on a 10-mesh screen.  
40 As clearly shown in Fig. 1, I prefer to

use coarser granular solids 7 on that portion of the butt exposed to the weather, and finer granular solids 8 on that portion of the armoring plate which underlies the shingle on the course above. For the finer solids the screenings from the coarser material may be used. The use of this finer material assists materially in conforming the protective plate to the taper form of the common shingle, besides creating value in an otherwise waste material.

As will be clear from the foregoing my armored shingle does not take fire readily since the bituminous matter which coats it must be heated to a very high temperature before it will give off enough inflammable vapor to make a blaze which will continue. It will be seen that dust, leaves or other matter collecting on a roof covered with my armored shingles will lodge against portions which are made fire-resistant, or which, thru melting of the armoring material become fire-resistant. On exposure to fire and a high degree of heat, a substantial, scab-like crust is formed by the armoring plate, which protects the part beneath by cutting off access of air. The "flying brand" hazard is greatly reduced by these crusts, which hold the coked wood in place until it is reduced to ash, or by cutting off access of air smother the glowing embers. Since my armored shingle tends to curl, contract or crack open under the influence of fire in much less degree than the ordinary shingle, the penetration of fire is greatly lessened.

It will also be recognized that roofs made of my armored shingles possess and preserve the individuality in the unit shingles thru the laying of narrow and wide shingles side by side in the same course. This avoids the mechanical regularity of the usual asphalt or asbestos shingle. It is quite obvious that the color of the individual shingles in any lot, of nominally the same color, may be varied sufficiently so that the appearance of deadness or flatness is avoided.

The armored shingle offers a unique opportunity to make use of fire-proofing chemicals in the wooden base of the shingle since all of the portions with which water comes in contact are protected so that leaching of the fire-proofing chemicals from the wooden shingle during the wet weather is avoided. Thus it becomes possible to impregnate the wood base with chemicals to increase its fire resistance, and such material tends to remain without being leached out during the entire life of the shingle.

It will be obvious that the mineral solid content of the bituminous vehicle of binding material may be varied to conform with varying conditions, but whatever the variation its primary purpose is to increase the amount of incombustible ash when de-

structive heat is applied to the shingle and to increase the resistance to fire under all conditions.

In Fig. 3 I have shown a modified form 5 of my shingle in which only the butt end and that portion adjacent the butt which is exposed to the weather is covered with the armoring plate. The priming coat 12 is applied over both top and bottom surfaces 10 adjacent the butt as shown, and protects the under side of the shingle from the weather. No granular matter is embedded in the armoring plate 13. This is probably the simplest form of my armored shingle.

In Fig. 4, I have shown another modified 15 form of my invention which differs from that shown in Fig. 1 by the inclusion of a layer of asbestos saturated with asphalt within the protective or armoring plate. 20 That is to say instead of incorporating the asbestos in the asphaltum in fiber form a sheet of asbestos is impregnated with asphalt and applied separately as shown. In this construction the priming coat 16 is applied as 25 already explained and the barbs are raised. Over the priming coat I apply a mixture 17 of asphaltum and crushed limestone, the asphaltum being of the general character already described, but preferably with a 30 penetration of 15 and a melting point of 175° F. 60 parts of the asphaltum are mixed with 40 pounds of limestone crushed to pass thru an 80 mesh screen, the asphalt being maintained at about a temperature of 35 35 35° during the mixing. While this coating is still plastic and adhesive the asphalt-saturated asbestos sheet 18 is rolled smoothly upon it. Preferably the asbestos is passed 40 over the butt end and for a short distance on the under side, so as to secure the end of the sheet against any tendency to loosen. The asbestos-saturated sheet may consist 45 of a sheet of asbestos weighing 9 pounds per 100 square feet, saturated with asphaltum thus bringing its weight to 12½ pounds per 100 square feet. Over the asbestos sheet is applied another layer 19 of asphaltum mixed with the crushed limestone previous-

ly used. A penetration of about 18 under the conditions already set forth and a melting point of about 200° F. will define an asphalt suitable for this purpose. It may be used without the admixture of mineral solids, but as already pointed out a greater quantity of ash is produced in burning 55 if the mineral matter is present. A mixture containing 80 parts of asphaltum and 20 parts of crushed limestone will give good results. While the coating is still plastic and adhesive the surface of coarse granular matter 21 and fines 22, is added in a manner similar to that already described.

As shown in Fig. 4, the wooden base may be a shake instead of a shingle. I have used the term shingle to include any rigid wooden 65 base used as shingles and shakes are used. Where the base is of the same thickness at butt and tip, I prefer to form my armoring coat a bit heavier at the butt end so that the armored portion at least presents a 70 tapered section similar to that of the standard shingle.

In Fig. 5 I have shown another modification which differs from that shown in Fig. 1 in the use of a layer 23 of asbestos saturated 75 with asphalt which extends from butt to tip of the shingle on the under side, and serves to resist the penetration of fire thru the layers of shingles for the longest possible time. After the priming coat is applied, an adhesive coat 24 of material similar to coating 17, described in connection with Fig. 4, is applied, and the asphalt-saturated asbestos sheet rolled smoothly upon it.

I claim:

A covering unit comprising a wooden base, a priming coat of low melting point bituminous compound on said base, barb raised on said coated base, and an armoring plate of high melting point bituminous compound united to said base by said priming coat and said barbs.

In testimony whereof, I have hereunto set my hand.

DOZIER FINLEY.